

## UNITED STATES PATENT OFFICE

WILLIAM H. MASON, OF LAUREL, MISSISSIPPI, ASSIGNOR TO MASONITE CORPORATION, OF LAUREL, MISSISSIPPI, A CORPORATION OF DELAWARE

## PROCESS OF MAKING PAPER PULP

No Drawing.

Application filed May 21, 1925. Serial No. 31,785.

My invention relates to a process of making paper pulp, and particularly to a process of making paper pulp of ligno cellulose material, by exploding same into a state of fine subdivision and treating such finely subdivided material with chemical reagents.

In the usual practice of making chemical paper pulp from wood chips, which always vary more or less in size, the smaller pieces and the outer surfaces of all the pieces are liable to be overtreated by the chemicals, whereas the inner portions of the larger pieces are frequently found incompletely digested. In the chip making a great deal of the comminuted wood has to be discarded as sawdust and the like prior to chemical treatment because of being too finely subdivided to be treated with the digester size chips. The chemical action is uneven from other causes. For example, there is extreme variation in the density of the wood treated, due to its irregular annular growth which leaves one part of the annular ring with extremely large and porous cells and another part dense, close and hard with comparatively few interstices through which the chemical can enter and react upon the material. Another variation in chemical access and reaction is due to the difference in the physical condition of the heart wood as compared with the sap wood. The heart wood has its cells largely closed and filled with resins and other waste material, while in the sap wood the cells are active and much more open. The difference in age of the various trees from which the wood is taken is also a factor in causing uneven chemical reaction with certain parts overdigested and others incompletely digested.

When wood is prepared for pulp making by grinding, the fibers are broken and torn and reduced in length and are not well adapted for the production of paper pulp from which strong, tough paper can be made.

According to the present invention in order to give the chemicals full access to the wood fibers and to provide enormously large surfaces for chemical attack, the wood or other ligno-cellulose material which is to be made use of for the production of paper pulp, is

exploded by being forcibly expelled from a high pressure chamber within which the material has been subjected to the penetrating action of a high pressure gas, such as steam, and whereby the ligno-cellulose material is reduced to very finely subdivided state, being in fact in large part reduced to its component ultimate fibers. With such treatment there is practically no reduction of fiber length, the fibers being practically all of their full natural length, and the exploded ligno-cellulose material is long fibered and well adapted for the production of paper pulp from which strong, tough paper can be made. Practically every bit of the wood is recovered as pulp, including the excessively dense and hard portions, such as knots, knurls and the like, which are thoroughly reduced to the fibrous state and available for making pulp.

In Patent No. 1,578,609 granted March 30, 1926, I have shown and described apparatus for performing the explosion operation. The explosion is preferably produced by high pressure steam which is, of course, at a correspondingly high temperature. By leading the exploded wood and exhaust steam into a digester or vessel in which the chemicals for pulp making are contained, substantially all the otherwise waste heat can be absorbed by the chemical liquid. The heat made use of to obtain the explosion can thus be practically all conserved.

According to the preferred embodiment of the invention the wood, chipped into pieces of about the size customarily made use of in chemical digesters, is introduced into a high pressure chamber and subjected to penetration by high pressure steam. After the pressure is balanced within and without the material to be exploded, an orifice is opened and the contents of the chamber discharged, the wood disrupting into a state of fine subdivision as it passes the orifice. The pressure is preferably maintained within the chamber during the explosion discharge so as to secure substantially uniform subdivision and disintegration from the first stages of the discharge right up to the completion thereof.

The pressures made use of in the explosion operation are in excess of 250# per square

inch. As the pressures are higher than this, more complete and better disintegration is obtained. A very desirably high state of disintegration has been obtained with steam at 500# per square inch.

I have found that when the wood used is of a uniform moisture content, desirably at or below the "fiber saturation point" of the wood, a most desirable condition is produced 10 for explosion. Less steam is required, on account apparently of there being less water to heat up to the high temperatures, and apparently the penetration of the steam into the interior of the wood is much more rapid and 15 complete and explosion thereof can be done much quicker with wood of substantially uniform low moisture content.

To obtain special conditions in the resulting fiber it may be desirable to preliminarily 20 dry the wood so that it is of uniform moisture content and desirably at or near the fiber saturation point. Predrying the wood enables the exploding to be done quickly and substantially avoids discolored products, 25 which may be produced when the wood is held too long under the high pressure steam.

After the wood is exploded and thereby reduced to fibrous state it is placed into a 30 digester and subjected to chemical digestion either of the acid or alkaline type in order to digest and remove all or part of the lignins and produce commercial cellulose pulp.

Desirably, although not necessarily, the exploded wood and exhaust steam is led directly 35 into the digester containing the chemical liquor so that the heat provided for the explosion step is not lost, but is in large part conserved. The time required in the digestion 40 operation is very largely reduced as compared with digesting treatment of the ordinary digester chips and considerable saving can be made in the reduced amount of chemical made use of. There is no substantial increase 45 in the amount of steam required and in some cases reduction of the steam is possible. There is more nearly the theoretical recovery of the complete cellulose content as pulp. A more uniform product is obtainable 50 apparently because of the very extensive exposure of the lignins and other non-cellulose components to the action of the chemical reagent. The pulp after digestion is ready for treatment in a beater, Jordan or the like apparatus 55 for the production of paper.

Instead of digesting the fibers completely as is required for very high grade pulp, a very desirable class of pulp is obtained by only partially digesting the exploded and 60 exposed fibers so that the lignin is removed to an extent from the individual fibers and it is possible to hydrate material so obtained by the usual process of hydration, such as beating, jordaning, etc.

65 Another mode of procedure in making pulp

with a combination of chemical and explosion treatment is to subject chips to complete or partial chemical treatment prior to explosion. Such treatment may be carried out in an enclosed chamber, the surplus chemical removed as by draining it out, and then the chips may be subjected in the chamber to very high steam pressure, such as pressure over 250# and preferably over 400# per square inch, and projected from the container as 70 described above, so that the resulting fiber is highly disintegrated. Many of the cellulose fibers have lost part or all of their coating of encrusting lignins so that they may be readily and more or less completely hydrated 75 by the ordinary beating process, and made available for a good grade of paper. If desired, the pretreatment with a chemical may be carried out in a separate vessel or digester prior to the introduction into and explosion 80 from the high pressure chamber. After explosion a further second treatment in a chemical digester may be resorted to, if desired.

The pretreatment with chemicals prior to explosion, when resorted to, may be of various 85 kinds. For example, discoloration produced by somewhat prolonged exposure to extra high pressure steam appears to be due to generation or liberation of acids, etc., and preliminary treatment with neutralizing 90 chemicals can be resorted to with advantage, especially when the steam pressures are extra high and discoloration of the product is undesirable.

95 I claim:

1. The process of making pulp, which consists in subjecting subdivided wood to chemical treatment in a chamber, removing surplus chemicals, subjecting the treated material to steam pressures in excess of 250# per square inch in said chamber, and discharging from said chamber at such pressure, whereby the material is exploded and thoroughly 105 disintegrated.

110 2. The process of making pulp, which consists in subjecting subdivided wood to chemical digestion in a chamber, removing surplus chemicals, subjecting the treated material to steam pressures in excess of 250# per square inch in said chamber, discharging said 115 chamber at such pressure, whereby the material is exploded and thoroughly disintegrated, and subjecting the predigested and exploded material to further chemical digestion.

120 3. The process of making pulp which consists in subjecting subdivided ligno-cellulose material to penetration by steam under pressure in excess of 250 pounds per square inch in a closed chamber, progressively discharging the ligno-cellulose material and steam through a constricted opening and leading the exploded material and exhaust steam into a liquid containing a chemical reagent for 125 digesting, whereby the heat of the steam used 130

for explosion is absorbed in the chemical reagent bath.

4. The process of making pulp, which consists in subdivision of wood into substantially chip form, subjecting same to partial chemical digestion, draining off the surplus liquid and exploding such pretreated wood into fibre by progressively discharging the same through a constricted opening from under pressure in excess of 250# per square inch.

5. The process of making pulp, which consists in subdivision of wood into substantially chip form, subjecting same to partial chemical digestion, draining off the surplus liquid, exploding such pretreated wood into fibre by progressively discharging the same through a constricted opening from under pressure in excess of 250# per square inch, and subjecting the partially digested and exploded fibrous material to further chemical digestion.

In testimony whereof, I have signed my name hereto.

WILLIAM H. MASON.